

1

3,050,391

## PHOTOGRAPHIC FILM WITH FINE GRAIN SILVER CHLORIDE UNDERLAYER

Thomas R. Thompson and Robert H. Clark, Binghamton, N.Y., assignors to General Aniline & Film Corporation, New York, N.Y., a corporation of Delaware  
No Drawing. Filed Dec. 30, 1957, Ser. No. 705,784  
5 Claims. (Cl. 96—61)

This invention relates to the manufacture of photographic film having improved sensitometric characteristics including speed and gradation. More particularly, it pertains to a photographic film having two emulsion layers including a novel underlayer emulsion of extreme low sensitivity.

In the process most widely used at the present time for the manufacture of photographic films of high sensitivity to light, a very sensitive silver halide emulsion is coated in a thin layer on a transparent plastic support. In cases when a high quality photographic reproduction is desired and also where a large degree of latitude in the photographic exposure must be available, a high speed emulsion layer is coated over another emulsion layer having a slightly slower speed, but of essentially the same magnitude. This arrangement of layers results in an extended straight line portion of the density-log exposure curve into the region of higher densities, but does not increase the over-all speed. It is important to note that the lower density range of speed of the top layer emulsion is not increased by the slower underlayer emulsion. Thus, the conventional practice of layer arrangements does not increase the sensitivity of the most sensitive element.

It is accordingly an object of this invention to provide a two layer film having improved photographic characteristics. Other objects will be apparent from the following description.

We have found that the speed of a two emulsion layer film is substantially increased by replacing the conventional lower layer by a novel undercoating consisting of a very fine grain, very slow speed emulsion. The photographic effect of the bottom layer is such as to increase the speed and gradient of the top layer.

In carrying out the invention, there is first coated upon the film base support a very slow speed emulsion. This slow speed emulsion is composed of a gelatin suspension of very small silver halide crystals having an average or median diameter on the order of 50 millimicrons. Even the largest particles do not exceed one micron in diameter as evidenced by the fact that all particles are invisible under the light microscope even when viewed under the highest magnification. Best results are obtained when the silver halide is essentially silver chloride. Since the crystals are small in size, there is afforded a very great surface area of silver halide for a given weight of silver halide since many minute crystals have a much larger surface than a few large crystals.

The small size of the crystals together with their large total surface area and their composition play an important part in this process. Thus, when a high speed bromoiodide silver halide emulsion, of the negative type, is coated over the slow speed emulsion, a photographic sensitometric evaluation gives a result of higher speed and gradient when compared to a single layer coating of the same high speed emulsion or when compared with a double layer film with two silver halide emulsion coatings in which the relative speeds of the lower and upper layers are essentially of the same magnitude.

The speed of the slow speed underlayer may be so slow that it requires an exposure of from 50 to 2000 times that of the more sensitive top layer. Assuming that the top layer has a relative speed of 100.0 (expressed in terms of reciprocal meter candle second to develop

2

a density of 0.2), the lower layers may have a speed between the range of 0.05 to 2.0. Thus, in this process, the bottom layer contains no developed silver even under conditions of exposure and development which give a high density in the top layer. This effect is clearly demonstrated by the examination under a microscope of cross sections made from a typical step tablet exposure suitably processed. Thus, a step of high density, as at the shoulder of the characteristic curve, shows a dense deposit of silver in the top layer, while the lower layer has no silver. This result is quite different from conventional commercial two layer films in which much silver density in both layers is observed in cross sections of exposed and developed high density areas. In this latter case, the purpose of the underlayer is to contribute density at higher exposure levels, thus extending the latitude of the product. In our invention, the underlayer contributes no density by virtue of developed silver in the underlayer itself.

The presence of the special underlayer of our invention does result in more silver density in the top layer after exposure and processing. A full scientific explanation of the mechanism by which our invention operates is not yet known. However, general considerations lead to two explanations, it being understood, of course, that these explanations are of a general nature and not intended to limit the scope of the invention.

One of these explanations assumes that some of the silver chloride in the lower layer is dissolved by the sulfite of the developer. This soluble silver product is free to diffuse into the top layer and supports a sub-latent image intensification.

An alternate theory postulates that after coating, the silver chloride of the bottom layer absorbs bromide ions from the top layer. It is known that highly sensitive silver bromoiodide emulsions contain soluble bromide ions which serve to stabilize the emulsion against fog or sensitivity changes during the film manufacture including the emulsion coating operation. Once the emulsion is coated on the support and water removed by drying, the bromide concentration increases. The high concentrations of bromide in the dried film may well reduce the film speed or reduce the development rate or increase the induction period of development.

It is now assumed by us that when the sensitive top layer is over-coated upon the fine grain, low speed silver chloride undercoating, soluble bromide ions may diffuse from the top layer and be adsorbed by the silver chloride. The adsorption of bromide ions by particles of silver chloride is essentially a surface reaction. Therefore, the greater surface of silver chloride afforded by the small particle size will promote a greater amount of bromide ion removal. Since bromide ions can diffuse throughout gelatin layers while silver chloride particles do not diffuse, there is reason to believe that at equilibrium the bromide ion concentration of the top layer can be reduced. The evidence available so far has not fully proven that either of the theories is correct, and it is, therefore, not intended that the scope of our invention be limited by the foregoing postulations.

The preferred type of undercoating emulsion is a silver chloride emulsion. A very slow speed silver chloride emulsion which is washed free of excess salts and has submicroscopic silver chloride particles within the size range specific is needed for that purpose. Since light sensitivity is not a factor, the silver chloride emulsion does not require a second digestion (after ripening). Ordinary photographic gelatins such as gelatin made from bone or hide are satisfactory. Silver bromide and silver bromoiodide emulsions can not be used. When they are coated in place of silver chloride as the undercoat, the effect of speed increase is not observed. Powerful organic stabilizers including the mercapto-substituted het-

erocyclic derivatives such as 2-mercaptopbenzothiazole or 2-mercaptop-5-phenyltetrazole when added to the undercoating drastically reduce or even eliminate the speed effect.

The silver chloride undercoating is most effective in causing speed and gradient increases in a medium or high speed silver bromoiodide overcoating. If overcoatings are used which have the speed of positive emulsions, little or no effect is observed. For this reason, an overcoating must be selected which belongs to the category of a high speed ammonia or boiled type emulsion of the type in which the silver halide in predominately silver bromide or silver bromoiodide with the iodide concentration not exceeding 5 mole percent based on the total weight of silver halide. The top layer may be optically sensitized and may, if desired, contain color formers fast to diffusion.

A wide variety of commercially available developers including those which are known by their trade names: Anasco 47, Anasco "Permadol" or Anasco "Liquadol" can be used satisfactorily for the development of our new materials. These developers are used for black and white development and contain hydroquinone and p-methyaminophenol (Metol) as the developing agents. Their composition is illustrated by Anasco A-47 which has the following formula:

|                                | Grams |
|--------------------------------|-------|
| Metol                          | 1.5   |
| Sodium sulfite, anhydrous      | 45.0  |
| Sodium bisulfite               | 3.0   |
| Hydroquinone                   | 6.0   |
| Sodium carbonate, monohydrated | 6.0   |
| Potassium bromide              | 0.8   |
| Water to make 1.0 liter.       |       |

Modifications in the composition of the developer, for instance, by adding excessive amounts of potassium bromide, or nitrobenzimidazole to the developers did not result in a noticeable increase in speed or reduction of fog enough to be of value.

The invention is further illustrated by the following examples, although it is to be understood that the invention is not to be restricted thereto.

#### EXAMPLE I

##### *Silver Chloride Emulsion*

| Part IA:        |             |       |  |
|-----------------|-------------|-------|--|
| Water           | milliliters | 225   |  |
| Sodium chloride | grams       | 25.5  |  |
| Gelatin         | do          | 16.5  |  |
| Part IB:        |             |       |  |
| Water           | milliliters | 225   |  |
| Sodium chloride | grams       | 19.65 |  |
| Part II:        |             |       |  |
| Water           | milliliters | 650   |  |
| Silver nitrate  | grams       | 60    |  |

Solutions IB and II were added simultaneously during the course of two minutes to solution IA with agitation at a temperature of 52° C. After a five minute period of digestion at 52° C., the mixture was precipitated by the addition of 90 grams of ammonium sulfate. Stirring was stopped and the precipitated silver chloride gelatin particles allowed to settle. Excess salts were removed by washing with decantation using dilution ratio of 1 to 4 and a total of three washes. After the final decantation, the precipitate was reconstituted with 75 grams of gelatin dissolved in 600 milliliters of water by agitating at 50° for twenty minutes. The resulting emulsion was made up to 1200 milliliters with water and found to have a pAg of 6.6 and a pH of 5.7.

The silver chloride emulsion was coated on a subbed cellulose acetate support to a thickness of 7 microns and, after drying, was overcoated with a medium speed silver bromoiodide emulsion at a thickness of 14 microns. A

70

control coating was prepared by coating the silver bromoiodide emulsion directly on the subbed support.

After a sensitometric exposure and processing, including 3 minute development in Anasco "Liquadol," fixing and washing, the following speed (1/e at density 0.2), gradient and fog values were obtained.

|         | Fog  | Speed | Gradient |
|---------|------|-------|----------|
| Control | 0.07 | 56    | 1.21     |
| Test    | 0.08 | 73    | 1.73     |

#### EXAMPLE II

Using the same silver chloride undercoat of Example I, an overcoating of 14 microns thickness was prepared using a high speed ammonia type silver bromoiodide emulsion:

|         | Fog  | Speed | Gradient |
|---------|------|-------|----------|
| Control | 0.09 | 138   | 1.94     |
| Test    | 0.16 | 180   | 2.00     |

#### EXAMPLE III

Using the same silver chloride undercoat of Example I, an overcoating was prepared using a high speed silver bromoiodide emulsion at a thickness of 15 microns.

|         | Fog  | Speed | Gradient |
|---------|------|-------|----------|
| Control | 0.07 | 120   | 0.99     |
| Test    | 0.08 | 142   | 1.35     |

#### EXAMPLE IV

As in Example III, a high speed silver bromoiodide emulsion was coated on a silver chloride emulsion undercoat. However, a polyethyleneoxide oleyl ether accelerator was added to the silver bromoiodide emulsion overcoating in the amount of 0.5 gram per liter of emulsion. The test coatings and the controls were developed for four minutes in Anasco "Permadol."

|                          | Fog  | Speed | Gradient |
|--------------------------|------|-------|----------|
| Control                  | 0.08 | 133   | 0.61     |
| Control plus accelerator | 0.12 | 180   | .68      |
| Test                     | 0.11 | 195   | .76      |
| Test plus accelerator    | 0.17 | 230   | .72      |

A silver chloride emulsion was prepared as follows:

|                 |             |      |
|-----------------|-------------|------|
| I. Water        | milliliters | 5900 |
| Sodium chloride | grams       | 165  |
| Gelatin         | do          | 875  |
| II. Water       | milliliters | 2400 |
| Silver nitrate  | grams       | 400  |

Part II was added during the course of one minute to part I at a temperature of 50°. After digesting for fifteen minutes, the mixture was chilled, shredded and washed to a conductivity of twenty  $\times 10^{-4}$  mho.

The silver chloride emulsion was coated on a film base support at a thickness of 7 microns and overcoated with a high speed silver bromoiodide emulsion of the ammonia type. After a sensitometric exposure and after processing one set of strips with Anasco "Liquadol" developer for three minutes, and the other set of strips with Anasco 47 developer for eight minutes, the following data was obtained.

|         | Development   | Fog  | Speed | Gradient |
|---------|---------------|------|-------|----------|
| Control | 3' "Liquadol" | 0.12 | 45    | 1.27     |
| Test    | 3' "Liquadol" | .17  | 140   | 1.33     |
| Control | 8' Anasco 47  | .16  | 54    | 1.14     |
| Test    | 8' Anasco 47  | .25  | 115   | 1.10     |

It will be seen from the above examples that the silver chloride underlayer emulsion is prepared in a simple manner. Other silver chloride emulsions, prepared by different procedures, may be used instead. In any case, the scientist skilled in the art can suitably adjust coating weights and amount of ingredients to achieve optimum results, provided the silver chloride particles are kept small in size for best results. The type of emulsion employed for the overcoating is not considered to be unusual. However, medium or high speed silver bromo-iodide emulsion containing from 1 to 5 mole percent iodide either of neutral or of the ammonium type are preferred.

Still other modifications of the invention will occur to persons skilled in the art. We, therefore, do not intend to be limited in the patent granted except as necessitated by the appended claims.

We claim:

1. A light-sensitive material carrying on a plastic transparent support in the following order, a subbing layer, a slow speed gelatinous silver chloride emulsion layer in which the silver chloride particles are of submicroscopic size and have a median particle size on the order of 50 millimicrons, and in direct contact with said silver chloride emulsion layer, a permanent high-speed gelatinous silver halide emulsion layer in which the silver halide emulsion is selected from the group consisting of silver bromide and silver bromoiodide emulsions and has a relative speed ranging from 45 to 138, the relative speed of said high-speed silver halide emulsion exceeding that of said silver chloride emulsion by a factor ranging from 50 to 2000, the speed of said lower silver chloride layer being so slow that no silver image is formed therein under conditions of exposure black and white development and fixing which give a high density silver image in the top layer, said relative speed being expressed in terms of reciprocal candle seconds to develop a density of 0.2.

2. In the process of forming a negative silver image in an imagewise exposed silver halide material, said process including the steps of black and white developing, fixing, washing and drying said silver halide material to form a permanent negative image therein, the improvement which consists of using as the light sensitive material a photographic element carrying on a plastic transparent support in the following order, a subbing layer, a slow-speed gelatin silver chloride emulsion layer in which the silver chloride particles are of submicroscopic size and have an average particle size of less than 50 millimicrons, and in integral contiguous contact with said silver chloride emulsion layer, a high-speed gelatin silver halide emulsion layer in which the silver halide emulsion is selected from the group consisting of silver bromide and silver bromoiodide emulsions, the photo-

40

1,303,635 Capstaff ----- May 13, 1919  
 2,202,026 Renwick ----- May 28, 1940  
 2,231,684 Schinzel ----- Feb. 11, 1941  
 2,258,187 Mannes et al. ----- Oct. 7, 1941  
 45 2,312,543 Goldfinger ----- Mar. 2, 1943  
 2,712,995 Weyde ----- July 12, 1955  
 2,725,296 Kendall ----- Nov. 29, 1955  
 2,927,024 Woodward et al. ----- Mar. 1, 1960

50

912,605 France ----- June 14, 1946

55 OTHER REFERENCES

Mees: "The Theory of the Photographic Process,"  
 pages 23 and 178, Macmillan Co., N.Y. (1954).

graphic effects of said improvement being such as to increase the effective speed and gradient of the silver image in the silver halide emulsion layer without the formation of a silver image in the silver chloride emulsion layer.

5 3. In the process of forming a negative silver image in an imagewise exposed silver halide material, said process including the steps of black and white developing, fixing, washing and drying said silver halide material to form a permanent negative image therein, the improvement which consists of using as the light sensitive material a photographic element carrying on a subbed transparent plastic support a gelatin silver bromoiodide emulsion layer having a relative speed ranging from 45 to 138 and between said emulsion layer and said support and in direct contact with said emulsion layer, a silver chloride gelatin emulsion layer in which the silver gelatin chloride particles are of submicroscopic size and have a median particle size of less than 50 millimicrons, said silver chloride emulsion having a relative speed between the range of 0.03 to 2.7, the speed of said silver chloride emulsion being insufficient to have a visible image formed therein under conditions of exposure and black and white development which give a high density silver image in said high-speed bromoiodide emulsion, said relative speed being expressed in terms of reciprocal candle seconds to develop a density of 0.2, the photographic effects of said improvement being such as to increase the effective speed and gradient of the silver image in the silver halide emulsion layer without the formation of a silver image in the silver chloride emulsion layer.

20 4. A process as defined by claim 2 wherein said silver halide emulsion layer contains a polyethylenoxide oleyl ether accelerator.

25 5. A process as defined by claim 3 wherein said silver halide emulsion layer contains a polyethylenoxide oleyl ether accelerator.

#### References Cited in the file of this patent

#### UNITED STATES PATENTS

1,303,635 Capstaff ----- May 13, 1919  
 2,202,026 Renwick ----- May 28, 1940  
 2,231,684 Schinzel ----- Feb. 11, 1941  
 2,258,187 Mannes et al. ----- Oct. 7, 1941  
 45 2,312,543 Goldfinger ----- Mar. 2, 1943  
 2,712,995 Weyde ----- July 12, 1955  
 2,725,296 Kendall ----- Nov. 29, 1955  
 2,927,024 Woodward et al. ----- Mar. 1, 1960

#### FOREIGN PATENTS

50 912,605 France ----- June 14, 1946

#### OTHER REFERENCES

Mees: "The Theory of the Photographic Process,"  
 pages 23 and 178, Macmillan Co., N.Y. (1954).